

May 19, 1936.

F. J. LANG

2,041,294

METHOD OF MAKING PAPER

Filed May 8, 1934

2 Sheets-Sheet 1



INVENTOR  
FRANK J. LANG

BY  
Frank J. Lang Jr.  
ATTORNEY

May 19, 1936.

F. J. LANG

2,041,294

METHOD OF MAKING PAPER

Filed May 8, 1934

2 Sheets-Sheet 2



INVENTOR  
FRANK J. LANG

BY

*Frank J. Lang*  
ATTORNEY

## UNITED STATES PATENT OFFICE

2,041,294

## METHOD OF MAKING PAPER

Frank J. Lang, Niagara Falls, N. Y., assignor to  
 International Paper Company, New York,  
 N. Y., a corporation of New York

Application May 8, 1934, Serial No. 724,536

9 Claims. (Cl. 92—21)

My invention relates to the manufacture of paper and more particularly to a method of, and apparatus for, producing paper having a filler such as calcium carbonate incorporated therein.

5 The principal object of my invention is to provide a method whereby the amount of filler retained in the fibres of the web is greatly increased, while a much smaller amount of alum than heretofore used is sufficient to bring about the objects 10 of the invention. Another object of my invention is to provide a method for the recovery of filler and color held in suspension in the white water leaving the machine and whereby to increase the efficiency of the usual suction pulp 15 filler.

A further object of my invention is to increase the color qualities of filled paper while obtaining the desirable objects of saving materials, increasing the retention of filler, and improving other 20 characteristics of filled paper.

A further object of my invention is to bring about the above desirable objects in a closed system wherein the materials carried away by the white water are reincorporated into the mix in 25 order that a greater amount of the materials may be incorporated into finished paper.

The invention may best be understood in connection with the following diagrammatic sketches wherein:

30 Fig. 1 is a schematic representation of a system taking white water from the paper machine and redistributing it back to various points, and showing one point of application of alum;

Fig. 2 is a similar schematic representation of 35 a system having the same general characteristics, wherein the alum is added at a different point;

Fig. 3 is a diagrammatic showing of the end 40 of a Fourdrinier machine opposite the head box, and illustrating the collection of white water from the wire.

In the making of filled papers it is common 45 practice to add a carbonate, such as calcium carbonate, or other carbonates of alkaline earth metals, to the mix in such proportions as to increase the opacity and brightness of the resulting paper. The amount of such carbonate retained in the felted fibres determines to a large extent the printing qualities of the paper, and thoroughness of incorporation tends to a large extent to prevent the formation of two-sided papers. Two-sided papers are usually the result of poor retention whereby the felt side of the 50 paper has more carbonate filler than the wire side.

My process eliminates two-sidedness to a great extent, as will appear.

In Fig. 3 the Fourdrinier wire 10 is shown passing over the usual couch roll 11, which in its preferred form is a foraminous roll having light 5 suction applied thereto. In advance of the couch roll are the usual suction boxes 12, and in advance of the suction boxes are the usual table rolls 13. The felted fibres are substantially formed into a web as they pass the table rolls, 10 and the suction boxes and couch roll remove as much water as possible before the web passes on to the press rolls, the dryers and the calendar stacks. The table rolls support the wire, and beneath these table rolls is the wire pit 14 where- 15 in most of the white water is collected. In advance of the table rolls are the usual head box, slice, apron, etc., and practically the entire amount of water is passed through the wire somewhere between the head box and the suc- 20 tion boxes. This water falls into the wire pit 14, from which some or all of the white water over- 25 flows into the usual overflow box 15. It is while the water is rapidly draining through the wire near the wet end of the machine that the greater 25 percentage of lost filler is removed from the mix and passes into the wire pit. The suction boxes and couch roll remove more of the filler, and the white water from these is collected in the couch 30 pit 16 which has an outlet 17 into the overflow 30 box 15. It can be seen that whatever goes to make up the white water in the way of fibres, 35 filler, or other matter, is collected in the over- 35 flow box 15 and passes into the white water tank shown in Figs. 1 and 2.

In Fig. 1 the overflow box 15 is utilized to add alum to the white water. This alum may be incorporated by injecting an alum solution or by placing an ingot of alum on the floor of the over- 40 flow box. The action of alum on carbonates 40 in producing aluminum hydroxide and the effect thereof on the fibres and web formation is well known.

From the white water tank the white water is 45 pumped into the flow box of a white water filter 45 wherein the chemicals soluble in water and the water are separated from the reclaimed stock. The coagulator, aluminum hydroxide, assists in flocculating the loose, minute fibres so that the filter may operate at its maximum efficiency to 50 remove the fibres. A screw conveyor may be utilized to start the reclaimed stock on its way to the filter chest.

The clear liquid passes into the clarified white 55 water sump and is pumped, either into a storage

5 tank for future use, or to various points in the paper process. The clarified water may be utilized as slush water for the washed soda pulp, as dilution water for a dropping bleacher, as dilution water for the bleacher dump chest, as dilution water on the flat screens, or wherever white water may be used.

10 Regardless of what point the clarified white water is returned into the system it will be at a point prior to the beaters and Jordans, and from there on it will be for a considerable time and to a much greater degree than heretofore thought possible incorporated into the mix. The mix may thus consist of fibres and the diluting liquids, 15 which in accordance with my invention will include reclaimed carbonate, alum and all of the products resulting from the chemical reaction of carbonates and alum. In the Jordans and in the beaters, these chemicals will be thoroughly 20 mixed or incorporated into close contact with individual fibres.

25 The white water which is drawn through the wire contains only a relatively small percentage of solids. This will be appreciated when it is realized that the pulp stream emerging from the slice has only one to one and a half parts solids in one hundred parts water. Inasmuch as the overwhelming bulk of solids is carried off in the form of the paper web, the dilution of white water 30 will be obvious. In point of fact, it frequently amounts to only one and one-half pounds of solids to one thousand gallons of white water. Under this condition there is little or no tendency on the part of the carbonate retained in the white 35 water in the overflow box to deteriorate the alum. Naturally, the clarified white water obtained after filtration represents very largely a mild alum solution. When this clarified white water is used to dilute the pulp, or for the purpose of dumping 40 the bleacher, or to wash the pulp in the Oliver filter or the flat screens, there is no ingredient present which can react adversely to the alum. As the result of the washing processes, the alum solution is drawn through the pulp over a 45 substantial period of time and results in thorough and uniform impregnation of the pulp with the alum solution. When pulp which has been so treated is placed in the beaters it has already been better and more thoroughly impregnated with 50 alum than could be done by any ordinary beating operation. When carbonate is then added to the beaters there is no opportunity for concentrated bodies of alum solution to come in contact with concentrated masses of carbonate, and as a result 55 there is no tendency to liberate large quantities of carbon dioxide due to reaction between the carbonate and the hydrolyzed alum.

60 Fig. 2 illustrates a system wherein even less alum is utilized, inasmuch as it is incorporated into the clarified white water at the white water sump, either by injecting a solution containing alum or by placing an ingot of alum in the sump. From there on the clarified white water passes to the same points of use and is taken into the 65 system prior to the beaters and Jordans.

67 In both systems the reclaimed stock from the filter is taken back into the system preferably through the first filter chest so that the reclaimed stock and whatever chemicals, such as aluminum hydroxide, may be carried with the reclaimed stock and thoroughly incorporated into the mix in the Jordans and beaters.

70 It will be apparent from the foregoing that the alum is evenly distributed throughout the system and is not injected into the mix in any con-

75 centrated amount in relatively small areas. The alum reacts to a certain extent with the reclaimed carbonate filler to form aluminum hydroxide which is a coagulator, flocculent and mordant. This makes certain that more fibres will be caused to adhere to each other due to the intimate association therewith of the aluminum hydroxide and as a result a stronger and finer interlocking of the fibres will be obtained. Each individual fibre will be more thoroughly coated 10 with the mordant and greater color retention will result.

15 In the beaters the fibres are more or less stretched and caused to curl so that they will tend to interlock with each other. If, as in my process, the alum is intimately associated with the fibres before the carbonate is added there will be more of a filling action, and more of the carbonate filler will be retained in the web itself due to the substantial reduction in size and number of interstices between fibres.

20 Whatever the correct theory of formation may be I have found that the resulting paper retains the filler to a greater extent than heretofore possible with a corresponding amount of filler, that less alum may be used since more of the alum actually used is put to practical effect, and that two-sidedness is avoided. It is also found that due to the long, intimate association and mixing action, the harmful effects of foaming are avoided, which 25 heretofore was thought to be impossible in any long mixing process. Excessive foaming is avoided due primarily to the fact that the pH value of the mix is such that the amount of carbon dioxide gas liberated by the action of the alum 30 on the calcium carbonate can all be absorbed by the calcium carbonate forming an acid carbonate. Hence, it can be said that there is no actual liberation of carbon dioxide gas. I have found that the resulting paper is entirely uniform and free 35 from lumps, spots and other defects, and that the paper has the desirable qualities to a high degree.

40 Other systems of arrangement of the various pumps, tanks and other portions of the system 45 may be utilized and I do not intend to be limited to those herein disclosed, except as set forth in the appended claims.

I claim:

45 1. In the method of making paper containing 50 a filler which is normally reactive with acidic material and wherein white water is filtered to recover stock therefrom, the steps of returning reclaimed stock to the beaters, and adding alum to the clarified white water which is thereafter 55 returned to the system prior to the beaters.

2. In the method of making paper, containing a filler which is normally reactive with acidic material, the steps of filtering the white water, returning the reclaimed stock to the beaters, adding alum to the clarified white water, and returning the clarified white water to the system prior to the beaters and washing the pulp therewith to thoroughly impregnate the fibres with alum.

3. In the method of making paper, containing a filler which is normally reactive with acidic material, the steps of adding alum to the white water, filtering the white water, returning the reclaimed stock to the beaters, and returning the clarified white water to the system prior to the 70 beaters, and washing the pulp therewith to thoroughly impregnate the fibres with alum.

4. In the method of making paper containing a filler which is normally reactive with acidic material, the step of washing the fibres with an 75

alum solution prior to their introduction into the beaters.

5. In the method of making paper containing a filler which is normally reactive with acidic material, the step of washing the fibres with an alum solution prior to their introduction into the beaters, and adding calcium carbonate to the alum-impregnated fibres in the beaters.

6. In the method of making paper containing 10 a filler which is normally reactive with acidic material, the improvement which consists of passing an alum solution through the pulp prior to its introduction into the beater.

7. In the method of making paper containing 15 a filler which is normally reactive with acidic material, the improvement which consists of passing an alum solution through the pulp prior to its introduction into the beaters and adding

calcium carbonate to the resulting alum-impregnated fibres in the beaters.

8. A method for the manufacture of paper containing an acid reactive filler comprising the steps of adding acidic material to the clarified white water, adding the said water to a fibrous mix at a point in the paper making system prior to the beaters, introducing said mix into a beater and then adding an acid reactive filler.

9. A method for the manufacture of paper, containing an acid reactive filler which comprises the steps of treating the white water with an acidic material, separating the fibres in the treated white water, returning said fibres to a beater, utilizing the white water to prepare a 15 fibrous mix, introducing said mix into the beater and thereafter adding an alkaline earth filler.

FRANK J. LANG.